

# UNITED STATES PATENT OFFICE.

EMILE BRONNERT, OF MULHOUSE, ALSACE-LORRAINE, FRANCE.

## MANUFACTURE OF ARTIFICIAL VISCOSE SILK.

1,374,718.

Specification of Letters Patent. Patented Apr. 12, 1921.

No Drawing.

Application filed September 8, 1920. Serial No. 408,987.

To all whom it may concern:

Be it known that I, EMILE BRONNERT, a citizen of the Republic of France, residing at 1 Quai du Barrage, Mulhouse, Alsace-Lorraine, France, have invented certain new and useful Improvements in the Manufacture of Artificial Viscose Silk, of which the following is a specification.

A process for spinning very fine threads from viscose solutions has been proposed, in which spinning baths containing aldehyde bisulfites or the reduction products thereof, ketone bisulfites or soluble condensation products of phenols with aldehydes and sodium-sulfites are employed.

Now it has been found that instead of adding these water soluble combinations to the spinning bath, it is preferable and more economical to add the various condensation products of phenols and aldehydes soluble in alkali, to the viscose itself, preferably prior to the ripening process, and to force the suitably ripened mixture into bisulfite baths for example.

### 25 Example.

10 kg. artificial resin produced from phenol and formaldehyde are dissolved in about 3.6 kg. caustic soda and 43 kg. water and then 1000 kg. freshly prepared raw viscose are added.

A homogeneous mixture of the above constituents is subjected to the usual ripening and then worked up into threads in the usual manner, use being made of a warm concentrated bisulfite bath. The feed of material is at the same time regulated to correspond to the desired fineness of the single threads and to the corresponding necessary drawing off speed. Apertures say of 0.10 mm. can be used, but also finer or larger ones may be employed, in taking in consideration the chosen viscosity of the viscose.

45 The concentration of the spinning baths must be the greater the finer the titre of the thread is desired. For ordinary threads of

7.5 deniers the technical bisulfite solution of about 30% sodium bisulfite content is sufficient. For the finer threads, for instance up to 1 denier and less, the concentration must be increased by the addition of solid sodium bisulfite or the more easily soluble ammonium bisulfite in a corresponding suitable manner. By increasing the temperature of the concentrated spinning baths to 70°, for instance, threads can be obtained directly washable after a short time, so that the troublesome subsequent fixing is done away with.

These products may be colored with the same dyes or coloring materials darker than the products obtained from raw viscose and without addition of other materials. A possible explanation is that the residue of the products precipitated out by the acid acts as a mordant. Also the resistance to water is somewhat higher than with viscose threads spun from viscose alone without the additions in question.

The broad idea of precipitating viscose in bisulfite baths, the concentration of which is inversely proportional to the thread fineness to be produced, is not herein claimed, as said matter is claimed broadly in my co-pending application, Serial No. 407,252, filed August 31, 1920.

I claim:

The process of producing artificial viscose silk threads up to 1 denier in fineness, consisting in that raw viscose with alkaline condensation products of phenols and aldehydes are spun in bisulfite baths, the concentration of the baths being inversely proportional to the thread fineness to be produced.

In witness whereof, I have hereunto signed my name in the presence of two subscribing witnesses.

EMILE BRONNERT.

Witnesses:

L. B. DE SALIS,  
N. SCHLUNNBERG.